

1

2,742,351

**STABILIZED HEATING OIL**

**Dilworth T. Rogers, Summit, and Harry W. Rudel, Roselle Park, N. J., assignors to Esso Research and Engineering Company, a corporation of Delaware**

No Drawing. Application June 7, 1951,  
Serial No. 230,443

4 Claims. (Cl. 44—76)

This invention concerns a fuel oil composition particularly characterized by the inclusion of salts of phosphorous, arsenic, antimony or bismuth, maintained in the fuel oil by means of a suitable detergent. In a preferred embodiment, the invention concerns cracked fuel oil compositions containing sodium phosphate dissolved in the oil with the aid of a detergent such as sodium petroleum sulfonate. The fuel oil compositions of this invention are advantageous in that they are effectively stabilized by inclusion of the additives indicated.

The invention is of application to hydrocarbon mixtures generally known as "fuel oils." Such hydrocarbon mixtures are employed in various burner systems as diesel fuels or as domestic and industrial heating oils. Fuel oils may be derived from petroleum by a variety of methods including the straight distillation from crude petroleum oil and thermal or catalytic cracking of petroleum oil fractions.

It has recently been observed that in the case of fuel oils consisting completely or in part of cracked stocks, these oils are characterized by undesirable instability. The instability is manifested by the formation of sediment after prolonged storage, particularly at elevated temperatures. Again, the instability of these fuel oils is evidenced by clogging of filters, orifices or fuel lines associated with burning systems in which the fuel oils are employed.

Consequently, this invention is of particular application to the preparation of fuel oil compositions which are made up at least in part of constituents derived from cracking operations. Such compositions may be effectively stabilized by employing additives herein disclosed.

Heating oils which may be stabilized by these additives are hydrocarbon mixtures of which more than about 10% consist of stocks derived from thermal or catalytic cracking operations. More precisely still, the base stocks may be characterized as petroleum fractions containing a proportion of cracked stocks greater than 10% and falling within A. S. T. M. specification D-975-48T for diesel fuel oils (grades Nos. 1-D to 4-D inclusive) and A. S. T. M. specification D-396-48T for fuel oils (grades Nos. 1 to 6 inclusive).

According to the present invention a small amount of a salt of certain of the group 5 elements is employed in the fuel oil to be stabilized. Salts of phosphorous, arsenic, antimony and bismuth may be employed. In particular, the alkali metal, alkaline earth or ammonium salts of these particular metals are to be employed. The benefits of this invention may be obtained in part by dispersing the indicated salts in finely divided form so as to permit the salts to remain in suspension in the oil. However, in the preferred practice of this invention, the

2

salts are maintained in oil solution with the aid of a suitable solubilizer or detergent. It has been found that an alkali or alkaline earth metal sulfonate which is oil soluble is effective in solubilizing the salts to be employed.

5 It is believed that a complex is formed between these oil soluble petroleum sulfonates and the salts of the group 5 elements serving to maintain the salts in solution. The preferred detergents are the alkali and alkaline earth metal sulfonates which are oil soluble. The oil soluble petroleum sulfonates of sodium and calcium are particularly contemplated for use. In the case of the alkaline earth metal sulfonates, the sulfonates of barium, calcium, strontium and magnesium are particularly preferred. Other detergents may be employed such as the metal soaps of the C<sub>16</sub> to C<sub>24</sub> fatty acids or of naphthenic acids. However, these detergents and other detergents which may be employed do not appear as effective as the metal petroleum sulfonates indicated.

20 Of the salts of phosphorus, arsenic, antimony and bismuth, which may be employed, the preferred salts are the salts of phosphorus, and particularly the sodium salts of phosphorus. Na<sub>3</sub>PO<sub>4</sub> presently appears to be the best of the sodium phosphates although Na<sub>2</sub>HPO<sub>4</sub>, NaH<sub>2</sub>PO<sub>4</sub>, Na<sub>4</sub>P<sub>2</sub>O<sub>7</sub> and Na<sub>3</sub>PO<sub>3</sub> have all been found to stabilize fuel oil. The present invention will be described with particular reference to the use of tri-sodium phosphate Na<sub>3</sub>PO<sub>4</sub> since this is the preferred compound. The anhydrous or hydrated forms of any of the described salts may be employed.

25 30 Only a very small proportion of a salt of arsenic, bismuth, antimony or phosphorus is to be included in the fuel oil. Expressing the proportion to be employed in terms of the anhydrous salts, the proportion to be used may vary from as little as about 0.0001 wt. percent up to about 0.1 wt. percent. In the preferred embodiment of this invention the salt of phosphorus, arsenic, bismuth or antimony is added to the fuel oil in the form of a complex with an alkali or alkaline earth metal petroleum sulfonate containing from about 2% to 20% of the salt 35 of one of these metals. In this case about 0.0005 to 5.0 wt. percent of this complex may be employed. Preferably however, the indicated complex is used in weight proportions of about 0.005% to 0.02%, based on the weight of the oil. Since these proportions are based on the use of anhydrous salts of these metals in the event a hydrated salt is employed, the proportions must be compensated in accordance with the water of hydration.

40 45 While, as indicated, actual solution of the selected salt in the oil is not necessary, it is preferred that the salt be dissolved in the fuel oil. A preferred procedure for incorporating the salt in heating oil is to prepare a complex with an oil soluble metallic sulfonate, e. g. of petroleum derivation and to dissolve the complex in mineral oil. This is accomplished by adding an aqueous solution of the salt, such as sodium phosphate to an oil soluble petroleum sulfonate, e. g. sodium or calcium sulfonate. Thereafter, the mixture is heated to a temperature of about 300° F. to completely dehydrate it. The phosphate in this case is in actual solution in the oil and no separation of the salt from the oil occurs until a critical concentration of the phosphate in the sulfonate is reached. A sodium sulfonate concentrate (for example, 65% sulfonate, 35% oil) can absorb up to about 20% of Na<sub>3</sub>PO<sub>4</sub>·12H<sub>2</sub>O. A 30% concentration of calcium sulfonate can absorb about the same quantity of the salt.

A concentrate of the sodium sulfonate phosphate complex prepared as indicated may then be employed in stabilizing fuel oil in the proportions formerly indicated.

In order to demonstrate the advantages and utility of the compositions of this invention, the following exemplary data are presented. In obtaining this data, a commercial heating oil was employed consisting of a blend of 20% to 30% catalytically cracked stock, 50% to 40% thermally cracked stock, and 30% virgin stock. Typical inspections of this type of oil are as follows:

|                                          |      |
|------------------------------------------|------|
| Grav., A. P. I.                          | 34.1 |
| Color, Tag Robinson                      | 1134 |
| Flash, ° F.                              | 158  |
| Sulfur (per cent)                        | 0.56 |
| Aniline point, ° F.                      | 130  |
| Neutralization No.                       | 0.07 |
| Dist. I. B. P. (° F.)                    | 342  |
| 10%                                      | 420  |
| 50%                                      | 484  |
| 90%                                      | 576  |
| F. B. P.                                 | 628  |
| Carbon residue on 10% bottoms (per cent) | 0.82 |

The sodium petroleum sulfonate employed in these tests was a concentrate of a sodium petroleum sulfonate having a molecular weight of about 467 in naphthenic lubricating oil in a weight proportion of about 50%. Three tests were used to evaluate the fuel oil compositions. Two of the tests involved a determination of the amount of sediment formed after 16 hours' storage at 210° F., and after 14 days of storage at 150° F. The third test involved the determination of rusting properties of the fuel oil composition to which 10% of water had been added, determined both in the water phase and in the oil phase. The results of these tests are indicated in the following table:

*Heating oil stability tests employing sulfonate-phosphate complex*

| Ratio:<br>$\text{Na}_3\text{PO}_4 \cdot 12\text{H}_2\text{O}$ / Na<br>Pet. Sulfonate | Concen-<br>tration<br>(Wt. Per-<br>cent) | Mg. Insoluble per<br>600 g. |                       | Rust Forma-<br>tion <sup>1</sup> |              |
|--------------------------------------------------------------------------------------|------------------------------------------|-----------------------------|-----------------------|----------------------------------|--------------|
|                                                                                      |                                          | 16 Hrs.<br>at 210° F.       | 14 Days<br>at 150° F. | Water<br>Phase                   | Oil<br>Phase |
| 0                                                                                    | 0.01                                     | 45                          | 22                    | None                             | None         |
| 0.067                                                                                | 0.01                                     | 12                          | 6                     | do                               | do           |
| 0.133                                                                                | 0.01                                     | 5                           | 3                     | do                               | do           |
| 0.20                                                                                 | 0.01                                     | 2                           | 1                     | do                               | do           |
| 0.266                                                                                | 0.01                                     | 2                           | 2                     | do                               | do           |
| 0.40                                                                                 | 0.01                                     | 2                           | 2                     | do                               | do           |
| 0                                                                                    | 0.0075                                   | 39                          | —                     | —                                | —            |
| 0.067                                                                                | 0.0075                                   | 12                          | —                     | —                                | —            |
| 0.133                                                                                | 0.0075                                   | 3                           | —                     | —                                | —            |
| 0.20                                                                                 | 0.0075                                   | 3                           | —                     | —                                | —            |
| 0.266                                                                                | 0.0075                                   | 3                           | —                     | —                                | —            |
| 0.40                                                                                 | 0.0075                                   | 4                           | —                     | —                                | —            |
| 0                                                                                    | 0.005                                    | 30                          | —                     | —                                | —            |
| 0.52                                                                                 | 0.005                                    | 6                           | —                     | —                                | —            |
| No additive                                                                          |                                          | 32                          | 21                    | Heavy                            | None         |

<sup>1</sup> Mild steel strip maintained in contact with oil sample containing 10% water for 52 days at room temperature.

As indicated in this table, the sodium phosphate maintained in the oil as a complex with sodium petroleum sulfonate was effective in all concentrations reported in stabilizing the fuel oil. In addition, the sodium phosphate, sodium sulfonate complex was effective in eliminating the corrosive properties of the fuel oil in the water phase. It is particularly significant that these data show that sodium petroleum sulfonate alone is not effective in overcoming the instability of the fuel oil, but the combination of sodium phosphate and sodium petroleum sulfonate is required.

Other experiments have been conducted to determine the operability of other of the phosphorus salts. These experiments are set forth in the following table; in which the indicated phosphorus salts were tested in the commercial heating oil formerly identified. In each case the salt of phosphorus was added to the commercial heating

oil in the form of a 50% concentrate of the phosphate salt in a lubricating oil vehicle.

*Effect of type of phosphate in complex*

| 5  | Phosphate Salt                                      | Ratio:<br>Salt / Na<br>Pet.<br>Sulfonate | Cone. of<br>Additive<br>(Wt.<br>Percent) | 16 Hrs. at<br>210° F.<br>(Mg. Insol./<br>600 g.) |
|----|-----------------------------------------------------|------------------------------------------|------------------------------------------|--------------------------------------------------|
| 10 | $\text{Na}_2\text{HPO}_4$                           | 0.08                                     | 0.01                                     | 1                                                |
|    | $\text{NaH}_2\text{PO}_4 \cdot \text{H}_2\text{O}$  | 0.08                                     | 0.01                                     | 1                                                |
|    | $(\text{NH}_4)_2\text{HPO}_4$                       | 0.08                                     | 0.01                                     | 3                                                |
|    | $\text{Na}_4\text{P}_2\text{O}_7$                   | 0.14                                     | 0.01                                     | 14                                               |
|    | $\text{Na}_3\text{PO}_4 \cdot 12\text{H}_2\text{O}$ | 0.20                                     | 0.01                                     | 1                                                |
|    | Sulfonate Alone                                     | 0.00                                     | 0.01                                     | 30                                               |
|    | Uninhibited                                         |                                          |                                          | 32                                               |

<sup>1</sup> Salts used in equivalent concentrations.

As shown in this table each of the salts of phosphorus solubilized by sodium petroleum sulfonate was effective in stabilizing the heating oil as demonstrated by the 16 hour stability test.

Further tests were then conducted to determine the operability of employing a salt of one of the indicated group 5 metals in a finely dispersed form in the absence of a solubilizer or detergent. 0.004 wt. per cent of sodium phosphate dodechydrate was dissolved in a small amount of water and added to the commercial heating oil formerly identified. This mixture was then heated while stirring and blowing with nitrogen to a temperature of 110° C. to drive off water. This served to leave the sodium phosphate in the heating oil in a finely dispersed form. The heating oil was then filtered and tested for stability employing the 16 hour stability test during which the oil was maintained at 210° F. In the case of the untreated oil at the end of the stability test, 32 mg. of sediment was formed per 600 g. of heating oil, and it was found that the color of the oil had degraded to a dark color and that the oil was turbid. In the case of the treated oil at the end of the stability test, it was found that only 16 mg. of sediment was formed per 600 g. of heating oil and that the color of the oil was light and the oil was clear. This data therefore shows that the finely dispersed salt, even without the presence of a solubilizer, is at least partially effective in stabilizing the heating oil.

Other experiments were then conducted to demonstrate the utility and operability of employing other of the salts of group 5 metals. Again the same formerly identified heating oil was employed and each of the salts was added to the heating oil in the form of a complex with sodium petroleum sulfonate. The data obtained is presented in the following table.

*Sodium salts of oxygen acids from group V elements*

| 55 | Salt              | Ratio:<br>Salt / Na<br>Pet.<br>Sulfonate | Cone. of<br>Additive<br>(Wt.<br>Percent) | 16 Hrs. at<br>210° F.<br>(Mg. Insol./<br>600 g.) |
|----|-------------------|------------------------------------------|------------------------------------------|--------------------------------------------------|
|    | Sodium Arsenite   | 0.16                                     | 0.01                                     | 1                                                |
|    | Sodium Arsenate   | 0.08                                     | 0.01                                     | 5                                                |
|    | Sodium Bismuthate | 0.14                                     | 0.01                                     | 28                                               |
|    | Sulfonate Alone   | 0.00                                     | —                                        | 30                                               |
|    | Uninhibited       |                                          |                                          | 32                                               |

<sup>1</sup> Salts used in equivalent concentrations.

As demonstrated by the data presented in this table, each of the salts was effective in improving the stability of the heating oil. It is particularly significant however that the salts of arsenic appear to be preferable to the salt of bismuth.

Finally, experiments were conducted in which a complex of sodium sulfonate and sodium phosphate as formerly described was added to a heating oil in combination with an alkaline earth metal, alkyl phenol sulphide. The particular compound employed was barium isoocetyl phenol sulphide. This data showed that stability of a heating oil may be enhanced by this three-component addi-

tive composition. The data obtained is presented in the following table.

*Sulfonate-phosphate complex<sup>1</sup> in combination with barium iso-octyl phenol sulphide*

| Additive (wt. percent Active Ingred.)                | 16 Hrs. at<br>210° F.<br>(mg. Insol./<br>800 g.) |
|------------------------------------------------------|--------------------------------------------------|
| 0.004% Ba Phenol Sulphide+0.01% Sulfonate-Phosphate  | 2                                                |
| 0.004% Ba Phenol Sulphide+0.01% Sulfonate            | 36                                               |
| 0.004% Ba Phenol Sulphide+0.005% Sulfonate-Phosphate | 2                                                |
| 0.004% Ba Phenol Sulphide+0.005% Sulfonate           | 27                                               |
| 0.002% Ba Phenol Sulphide+0.01% Sulfonate-Phosphate  | 1                                                |
| 0.002% Ba Phenol Sulphide+0.01% Sulfonate            | 30                                               |
| Uninhibited                                          | 32                                               |

<sup>1</sup> Ratio:  $\text{Na}_3\text{PO}_4 \cdot 12\text{H}_2\text{O}$  to Sodium Petroleum Sulfonate = 0.20.

In accordance with this invention therefore, an alkali, alkaline earth metal or ammonium salt of phosphorus, antimony, arsenic or bismuth is to be incorporated in a cracked fuel oil in minor proportions. It is preferred to maintain one or more of these salts in the fuel oil by means of a solubilizer or a detergent. The preferred detergent constitutes an alkali or alkaline earth metal oil soluble petroleum sulfonate. In addition, it is particularly contemplated that other compounds may be included in the heating oil composition such as an alkaline earth metal alkyl phenol sulphide. It is apparent that other conventional additives ordinarily employed in a fuel oil may also be incorporated in the fuel oil compositions of this invention.

What is claimed is:

1. The process of stabilizing a heating oil constituting a petroleum fraction containing a proportion of cracked stocks greater than 10% and falling within A. S. T. M. specification D-975-48T and A. S. T. M. specification D-396-48T, which comprises incorporating in the said petroleum fraction about 0.0001 to 0.1 weight percent of a compound selected from the group consisting of the alkali

metal, alkaline earth and ammonium phosphates, arsenites, arsenates and bismuthates.

2. The process defined by claim 1 in which the said compound is incorporated in the heating oil by formation of a complex with a compound selected from the group consisting of the alkali metal and alkaline earth metal oil-soluble petroleum sulfonates.

3. A heating oil composition comprising a petroleum fraction containing a proportion of cracked stocks greater than 10% and falling within A. S. T. M. specification D-975-48T and A. S. T. M. specification D-396-48T, and containing about 0.0005 to 5 weight percent of a compound selected from the group consisting of the oil-soluble alkali and alkaline earth metal petroleum sulfonates, and including about 2% to 20% of trisodium phosphate based on the said sulfonate.

4. A composition consisting essentially of a distillate heating oil containing more than about 10% of cracked constituents and containing about 0.0001 to 0.1 weight percent of a compound selected from the group consisting of the alkali metal, alkaline earth metal, and ammonium phosphates, arsenites, arsenates, and bismuthates, together with a minor and solubilizing proportion of a compound selected from the group consisting of the alkali metal and alkaline earth metal oil-soluble petroleum sulfonates.

References Cited in the file of this patent

UNITED STATES PATENTS

|    |           |               |               |
|----|-----------|---------------|---------------|
| 30 | 2,137,727 | Quirke        | Nov. 22, 1938 |
|    | 2,301,370 | Cook et al.   | Nov. 10, 1942 |
|    | 2,409,687 | Rogers et al. | Oct. 22, 1946 |
| 35 | 2,527,987 | Caron et al.  | Oct. 31, 1950 |
|    | 2,623,016 | Mertes        | Dec. 23, 1952 |

OTHER REFERENCES

Monsanto Technical Bulletin, No. P-24, June 15, 1940, 6 pages, Monsanto Chemical Co., St. Louis, Mo.  
Industrial and Engineering Chemistry, vol. 23, No. 5, 40 pages 470-474, Dec. 9, 1930.